

1

2,881,121

## ELECTROPLATING

Donald G. Foulke, Watchung, Otto Kardos, Red Bank, and Herman Koretzky, Belleville, N.J., assignors to Hanson-Van Winkle-Munning Company, a corporation of New Jersey

No Drawing. Application March 14, 1957  
Serial No. 645,922

11 Claims. (Cl. 204—52)

This invention relates to electroplating and, more particularly, to electrodepositing copper from an aqueous alkaline cyanide copper plating bath. The invention is based on our discovery that both alkali-soluble trivalent bismuth compounds and water-soluble acetylenic compounds, when incorporated in a copper plating bath in conjunction with selenium compounds, are capable of promoting the formation of excellent bright and ductile electrodeposits of copper over a wide current density range.

The electrodeposition of copper from an alkaline cyanide plating bath containing only an alkali-soluble selenium compound as the brightening additive generally produces electroplates which are bright over a relatively narrow current density range, e.g. between 2 and 10 amperes per square foot, while semi-bright and even hazy deposits are formed at current densities below and above these limits. When, however, a small quantity of either an alkali-soluble trivalent bismuth compound or a water-soluble acetylenic compound is incorporated in the plating bath together with a selenium compound, the brightening capacity of the bath is markedly extended, and the electrodeposit is bright and frequently brilliant over a very wide current density range.

The brightening capacity may be extended still further by adding certain nitroxy compounds to the plating bath. These compounds are effective in alkaline copper cyanide baths which contain a bismuth compound, an acetylenic compound, or a titanium compound in addition to a selenium compound. The nitroxy compounds extend the bright current density range to a remarkable degree.

The process of our invention is accomplished most advantageously by using an alkali cyanide copper plating bath in which both the concentration of copper and of cyanide, as well as the ratio of copper concentration to cyanide concentration, are within the limits generally employed for standard copper electroplating operations. Such baths usually contain from 20 to 75 grams per liter of copper and from 45 to 145 grams per liter of an alkali metal cyanide. In this plating bath, we generally employ from 0.01 to 20 millimoles per liter of an alkali-soluble selenium compound, and from about 0.005 to about 200 millimoles per liter of the bismuth compound or acetylenic compound (or titanium compound, when a nitroxy compound is also present). A nitroxy compound can be used with advantage in combination with either a bismuth compound or an acetylenic compound, as well as in combination with a titanium compound. In addition small quantities of auxiliary compounds, such as various nitriles and water-dispersible wetting agents, may also be incorporated in the bath.

In the case of the trivalent bismuth compounds, only relatively small quantities are required in the plating bath, especially when they are used in conjunction with a selenium brightener. In general, concentrations of the trivalent bismuth compound as low as 0.005 millimole

2

per liter (0.002 gram per liter of bismuth) are effective, though for optimum results it is usually preferable to employ at least 0.025 millimole per liter. In general the trivalent bismuth compound may be used over a relatively wide range in concentrations, but there is no great advantage in using more than about 1 gram per liter, and in most plating baths substantially the full benefit of its presence is achieved with concentrations of 0.02 gram per liter or even less.

10 Any trivalent bismuth compound capable of being dissolved in weakly alkaline media may be successfully employed in the plating bath. Various bismuth salts, such as bismuth citrate, bismuth subsalicylate and bismuth tartarate, have been used successfully, but most bismuth salts are insoluble or dissolved with great difficulty in alkaline solution. We have obtained particularly satisfactory results using a trivalent bismuth coordination compound having at least one ligand selected from the group consisting of polyols and hydroxycarboxylic acids. 15 These compounds are soluble in water and generally stable in alkaline solution. They may be prepared by slowly adding a bismuth salt to an aqueous solution of the polyol or hydroxycarboxylic acid. Although the precise structure of the coordination compound is unknown, 20 the cluster of hydrophilic ligands surrounding the bismuth nucleus allows the complex to be solvated by water. Thus, bismuth coordination compounds containing ligands of hydroxycarboxylic acids, such as gluconic acid, or 25 those prepared from polyols such as sorbitol and glycerol, 30 are particularly effective when incorporated in the plating bath with an alkali-soluble selenium compound.

When an acetylenic compound is used in the bath, it preferably is above 1 millimole per liter, and for optimum results it is usually preferable to employ at least 10 millimoles per liter. There appears to be no critical upper limit to the concentration of the acetylenic compound save solubility, but there is no great advantage in using more than about 200 millimoles per liter, and in most plating baths substantially the full benefit of its presence is achieved with 100 millimoles per liter or even less.

While any water-soluble acetylenic compound may be employed in the plating bath to produce bright copper deposits in accordance with the invention, we have obtained particularly satisfactory results using either oxygen-containing acetylenic compounds (especially acetylenic alcohols) or acetylenic amine compounds. Compounds from among the oxygen-containing acetylenic group which have been found to be very satisfactory are 40 those which have the formula



55 in which  $\text{R}_1$  and  $\text{R}_2$  are substituents selected from the group consisting of hydrogen and alkyl and hydroxy-substituted alkyl radicals,  $\text{R}_1$  is a substituent selected from the group consisting of hydroxy, hydroxymethyl, methoxy, hydroxyethyl, ethoxy, and hydroxyethoxy radicals, 60 and  $\text{R}_2$  is a substituent selected from the group consisting of hydrogen, halogen, diethylaminoethyl, morpholino-methyl, alkyl, alkenyl, alkynyl, and hydroxy-, methoxy- and ethoxy-substituted alkyl, alkenyl, and alkynyl radicals. When used in the plating bath in conjunction with a selenium compound, these water-soluble oxygen-containing acetylenic compounds produce bright electrodeposits at current densities ranging from 1 to 100 amperes per square foot.

70 The acetylenic amines function particularly effectively at the higher current densities. As a general rule, the acetylenic amines are less soluble in an alkaline

media than the oxygen-containing acetylenic compounds. Among the various acetylenic amines that have been used successfully in conjunction with the selenium compounds are those water-soluble compounds of the group consisting of monoacetylenic primary monoamines, monoacetylenic polyamines, polyacetylenic monoamines, polyacetylenic polyamines, acetylenic alkanolamines, and acetylenic ammonium compounds.

The compounds listed in Table I are examples of water-soluble acetylenic compounds which have been used successfully in plating baths containing selenium compounds. As indicated previously, these compounds are advantageously used in concentrations from 1 to 200 millimoles per liter.

TABLE I  
Water-soluble acetylenic compounds for bright copper plating

| Compound                             | Structure                                                                                                              |
|--------------------------------------|------------------------------------------------------------------------------------------------------------------------|
| 2-Butyne-1,4-diol                    | $\text{HO}-\text{CH}_2-\text{C}\equiv\text{C}-\text{CH}_2-\text{OH}$                                                   |
| Propargyl alcohol                    | $\text{HC}\equiv\text{C}-\text{OH}, \text{OH}$                                                                         |
| Dipotassium acetylenedicarboxylate   | $\text{KOOC}-\text{C}\equiv\text{C}-\text{COOK}$                                                                       |
| 1,4-Dimethoxy-2-butyne               | $\text{H}_3\text{COOCH}_2-\text{C}\equiv\text{C}-\text{OCH}_3, \text{OCH}_3$                                           |
| 2,4-Hexadiyne-1,6-diol               | $\text{HOCH}_2-\text{C}\equiv\text{C}-\text{O}-\text{O}-\text{CH}_2\text{OH}$                                          |
| 1-(N,N-diethyldiamino)-2-butyne-4-ol | $(\text{CH}_3\text{CH}_2)_2\text{N}-\text{CH}_2-\text{C}\equiv\text{C}-\text{CH}_2\text{OH}$                           |
| Dimethyl 3-hexynoate                 | $\text{H}_3\text{COOCCH}_2-\text{C}\equiv\text{CCH}_2-\text{OOOCCH}_3$                                                 |
| 1-Butyn-4-ol                         | $\text{HC}\equiv\text{C}-\text{OH}, \text{CH}_3\text{OH}$                                                              |
| 2-Methyl-3-hydroxyethoxy-1-butyne    | $\text{H}_3\text{O}(\text{CH}_2)-(\text{OC}_2\text{H}_5\text{OH})-\text{C}\equiv\text{OH}$                             |
| 3-Methyl-1-butyne-3-ol               | $\text{OH}-\text{C}(\text{CH}_3)-(\text{OH})\text{C}_2\text{H}_5\text{OH}$                                             |
| Propargyl amine                      | $\text{HC}\equiv\text{CCH}_2\text{NH}_2$                                                                               |
| 1,4-(N,N-diethyldiamino)-2-butyne    | $(\text{CH}_3\text{CH}_2)_2\text{N}-\text{CH}_2-\text{C}\equiv\text{C}-\text{OCH}_2\text{N}(\text{CH}_3\text{CH}_2)_2$ |
| 3-Amino-3-methyl-1-butyne            | $\text{CH}_3\text{C}(\text{CH}_3)-(\text{NH}_2)\text{C}\equiv\text{OH}$                                                |
| 3-Amino-3-ethyl-1-butyne             | $\text{CH}_3\text{C}(\text{CH}_2\text{CH}_3)-(\text{NH}_2)\text{C}\equiv\text{OH}$                                     |

Selection of a selenium "primary" brightener addition agent for inclusion in the plating bath may be made from either organoselenium compounds or selenium salts, including selenides, selenites, selenates and selenocyanates. Although these selenium compounds may be used over a very wide range of concentrations, they are preferably employed in an amount to yield from 0.001 to 0.5 gram per liter of selenium; or, expressed in equivalent weights, we use from about 0.01 to about 20 millimoles of the selenium compound per liter.

It is generally possible to improve the brilliance of the electroplates, and to further broaden the current density range over which bright deposits are formed, by incorporating a small amount of an alkali-soluble nitroxy compound in the plating bath. When employed in a plating bath with a selenium compound and a bismuth compound or acetylenic compound, or an alkali-soluble titanium compound, the nitroxy compound extends to a remarkable degree current density range over which bright deposits can be formed. The nitroxy compounds employed all contain, as their common structural feature, an ionic moiety represented by the formula



in which  $\alpha$  is an atom selected from the group consisting of oxygen and disubstituted carbon atoms, and  $\beta$  is a member of the group consisting of an electron pair and a coordinately bonded oxygen atom. Thus, when  $\alpha$  is an oxygen atom, the nitroxy compound may be either an inorganic nitrite ( $\beta$ =an electron pair) or an inorganic nitrate ( $\beta$ =a coordinately bonded oxygen atom), since these compounds dissolve in alkaline solution to form nitrite and nitrate ions respectively. On the other hand, when  $\alpha$  is a disubstituted carbon atom, the nitroxy compound may be either an oxime ( $\beta$ =an electron pair) or a nitroalkane ( $\beta$ =a coordinately bonded oxygen atom). When organic nitrates and nitrites are used, they should be salts whose cations do not precipitate in the alkaline cyanide solution and do not exert any deleterious effect. Especially satisfactory nitrates and nitrites are those of the alkali metals, magnesium, ammonium and copper. Among the nitroalkanes that may be used, nitromethane

is particularly satisfactory, and aldoxime and dimethylglyoxime are examples of satisfactory oximes.

However, any such nitroxy compound, which is capable of being dissolved in weakly alkaline media and does not undergo decomposition in the presence of hydroxide ions may be successfully employed in the plating bath. We generally prefer to employ a nitroxy salt of an alkali metal, i.e. an alkali metal nitrate or nitrite; and, we have found that in general the full benefit of their presence is achieved with amounts in the range from 7.5 to 45 grams per liter.

In all, three classes of "secondary" brightener addition agents have been successfully employed in the plating bath in conjunction with a selenium "primary" brightener ad-

ditive and the nitroxy compound. These include, in addition to the previously mentioned alkali-soluble trivalent bismuth compounds and alkali-soluble acetylenic compounds, the alkali-soluble titanium compounds which are described in the copending application of Donald G. Foulke and Otto Kardos, Serial No. 582,661, filed May 4, 1956, now United States Patent No. 2,848,394, granted August 19, 1958. Included among the titanium compounds capable of being dissolved in weakly alkaline media and which can be used in combination with a selenium compound and a nitroxy compound are various titanium salts, such as potassium titanate, titanium lactate and potassium titanium oxalate, in which the titanium moiety may be either in the cationic or anionic portion of the compound. Particularly satisfactory results have been obtained, however, using titanium coordination compounds having at least one ligand which is a polyol or alkanolamine. These titanium coordination compounds are soluble in water and generally stable in alkaline solution; they are prepared by condensing a titanium halide together with an alkoxide of the polyol or alkanolamine. Although the titanium compounds may be employed in the bath in concentrations as low as 0.005 and as high as 200 millimoles per liter, they are preferably used in concentrations ranging from 0.5 to 25 millimoles per liter.

The lustre and brilliance of the electroplate and the range of optimum plating conditions may be still further broadened by incorporating a small amount of various auxiliary agents in the plating bath. Wetting agents are among the most useful of these auxiliary agents. We have had particular success by adding to the plating bath a polyoxy compound having the formula



in which  $\text{R}_1$  is a substituent selected from the group consisting of hydrogen and methyl,  $\text{R}_2$  and  $\text{R}_3$  are substituents selected from the group consisting of hydroxy, alkoxy, thioalkoxy, phenoxy, alkylphenoxy, thiophenoxy, alkylmercapto, and carboxamido, and  $n$  is an integer from 6 to 60. These polyoxy compounds are, of course, polyoxyethylene or polyoxypropylene glycol, and the condens-

sation products of ethylene or propylene oxide together with alcohols, thioalcohols, phenols, thiophenols and amides. The polyoxy compound may be added at any time during the preparation of the plating bath, and may be used in concentrations in the range from 0.05 to 20 grams per liter.

Alkali-soluble nitriles are examples of other auxiliary brightening agents which may be successfully employed in the plating bath together with either a bismuth or an acetylenic compound and an alkali-soluble selenium compound. Table II sets forth several examples of such nitriles which have been used successfully in embodiments of this invention. The concentration values set opposite each compound in Table II were found to give good results when that compound was used in combination with an alkali-soluble "primary" selenium brightening compound and either a trivalent bismuth compound or an acetylenic compound. These concentrations, however, do not necessarily indicate optimum, or maximum or minimum concentrations. In general, from 0.05 to 20 grams per liter of an alkali soluble nitrile may be used in the bath.

Indeed, the brightening agents described above function particularly well in a sodium plating bath, especially at the higher concentrations of copper and at higher temperatures.

Table III illustrates the effect exerted by trivalent bismuth in extending the brightening capacity of a copper plating bath containing a selenium "primary" brightener. This table summarizes a series of tests which were carried out on a typical plating bath containing a representative alkali-soluble selenium compound, alone and in combination with a trivalent bismuth compound. In each of these particular examples, a typical alkaline cyanide copper plating bath, containing 48 grams per liter of copper (as metal), 9 grams per liter of free potassium cyanide, 30 grams per liter of potassium hydroxide, and 30 grams per liter of potassium sodium tartarate, was used. Plating operations in each example were carried out in a Hull test cell so that the effect of a wide range of current densities could be observed. The electrodeposits were formed on brass cathodes at a temperature of 150° F.

TABLE III  
*Effect of trivalent bismuth additives on bright copper plating*

| Selenium Compound            | Conc.<br>(Gm./L.) | Bismuth<br>Tartarate<br>(Gm./L.) | Character of Deposit                                                                                                   |
|------------------------------|-------------------|----------------------------------|------------------------------------------------------------------------------------------------------------------------|
| Potassium selenocyanate..... | 0.003             |                                  | Hazy bright in the lower $\frac{1}{4}$ of the current density range; matte in the current density range below 2 a.s.f. |
|                              | 0.008             | 0.0054                           | Fully bright over the entire current density range including the range below 2 a.s.f.                                  |
| Potassium selenate.....      | 0.06              | 0.0054                           | Semi-bright from 2-12 a.s.f.                                                                                           |
|                              | 0.08              | 0.0054                           | Improved brightness intensity over the entire current density range; fully bright from 2-8 a.s.f.                      |
| Potassium selenite.....      | 0.064             |                                  | Milky and semi-bright over most of the current density range.                                                          |
|                              | 0.064             | 0.0054                           | Increased intensity in brightness, and especially in low current density range.                                        |
| Potassium selenide.....      | 0.02              |                                  | Hazy and semi-bright up to about 14 a.s.f.                                                                             |
|                              | 0.02              | 0.0054                           | Improved brightness with considerably less haze over entire current density range.                                     |

<sup>1</sup> As the sorbitol complex.

TABLE II

*Nitriles used in bright copper plating*

|                                           | Grams per liter |
|-------------------------------------------|-----------------|
| Succinonitrile .....                      | 0.05 to 0.5     |
| Dicyandiamide .....                       | 0.12            |
| $\beta, \beta'$ -Oxydipropionitrile ..... | 0.12            |
| Potassium dicyanoguanidine .....          | 0.12            |
| $\beta$ -Sulfopropionitrile .....         | 0.12            |
| Sodium dicyandiamide .....                | 0.12            |

A conventional alkaline-cyanide copper plating bath, to which the primary, secondary and auxiliary brightening agents may be added for making up a plating bath in accordance with this invention, customarily has the following composition:

|                                 | Ounces<br>per<br>Gallon | Grams<br>per<br>Liter |
|---------------------------------|-------------------------|-----------------------|
| Copper (as metal).....          | 8 to 10                 | 20 to 75              |
| Potassium cyanide (total).....  | 6 to 10                 | 45 to 120             |
| Potassium hydroxide.....        | 1 to 5                  | 7.5 to 40             |
| Potassium sodium tartarate..... | 3 to 6                  | 15 to 45              |
| Potassium carbonate.....        | 0 to 15                 | 0 to 110              |

The tartarate (Rochelle salt) and carbonate, while preferred, are optional ingredients and can be omitted. Although sodium salts may be used interchangeably for the potassium salts, the use of the potassium plating bath has found increased favor in recent years. The addition agents described in the invention, however, are equally applicable to both sodium and potassium plating baths.

Examples I to IV below illustrate the effect exerted by water-soluble acetylenic compounds on the brightening capacity of copper plating baths containing selenium compounds. Table IV lists the basic compositions of two plating baths which were employed in carrying out these and other examples of the invention that are set forth below.

TABLE IV  
*Bath concentrations in grams per liter*

|                                 | Bath A | Bath B |
|---------------------------------|--------|--------|
| Cuprous cyanide.....            | 48.00  | 66.75  |
| Potassium cyanide (free).....   | 9.0    | 9.0    |
| Potassium hydroxide.....        | 30.0   | 30.0   |
| Potassium Sodium Tartarate..... | 30.0   | 30.0   |

In each of the following examples demonstrating the effect of the acetylenic compounds, the electrodeposit was formed in a Hull test cell so that the effect of a wide range of current densities could be observed. In each case, the electrodeposits were formed on brass cathodes at temperatures varying between 60° and 68° C., with agitation provided where indicated.

## EXAMPLE I

To a standard copper plating bath (Bath A of Table II) was added 0.003 gram per liter of potassium selenocyanate, and copper was electrodeposited on a test panel, without agitation, at a temperature of 68° C. The deposit was bright only at current densities between 2 to 10 amperes per square foot, and was noticeably hazy below 2 amperes per square foot.

Upon the addition of 1 gram per liter of 2-butyne-1,4-diol to this bath, a very bright deposit was obtained under identical plating conditions over a current density range between 0 and 20 amperes per square foot. When air and mechanical agitation were provided, bright deposits were obtained between 10 and 40 amperes per square foot.

#### EXAMPLE II

Using a standard copper plating bath (Bath A) which contained 0.13 gram per liter of sodium selenite, a bright electroplate was deposited between 2 and 10 amperes per square foot on the test panel in a Hull cell operated at 68° C. When 1 gram per liter of 2-butyne-1,4-diol was added to this bath, a bright deposit was obtained over the range from the lowest observable current density to 20 amperes per square foot.

#### EXAMPLE III

A bright copper deposit was formed at current densities between 2-10 amperes per square foot on a polished brass panel in a Hull cell, using a plating bath and plating conditions similar to those described in Example I, with the sole exception that 0.3 gram per liter of sodium selenite was used in the bath in place of potassium selenocyanate. By adding 1 gram per liter of 2-butyne-1,4-diol to the bath, the electrodeposit was fully brilliant from the lowest observable current density to 20 amperes per square foot.

#### EXAMPLE IV

The acetylenic compounds have also proved exceptionally effective in copper plating baths containing selenide brightening additives. Using a standard copper plating having the basic composition of Bath B and containing 0.002 gram per liter of sodium selenide and 1 gram per liter of 2-butyne-1,4-diol, deposits formed on test panels at a bath temperature of 68° C., without agitation, were fully bright current densities from the lowest observable value to 25 amperes per square foot. Similarly, when 0.45 gram per liter of propargyl alcohol was added to the bath in place of 2-butyne-1,4-diol, and the concentration of sodium selenide increased from 0.002 to 0.004 gram per liter, a bright copper electroplate was formed, without agitation, over the current density range from the lowest observable value to 20 amperes per square foot. The substitution of other acetylenic compounds, notably 2-methyl-3-butyne-2-ol, 2,4-hexadiyne-1,6-diol, dipotassium acetylenedicarboxylate, dimethyl ester of 2-butyne-1,4-dicarboxylic and 3-methyl-1-butyne-3-ol in equivalent amounts, also produced bright copper deposits at all current densities up to 20 amperes per square foot.

The effect exerted by the nitroxy compounds in extending the bright plating range was demonstrated in a series of tests carried out using typical plating baths containing representative primary and secondary brightening agents, with and without the addition of an alkali-soluble nitroxy compound. In each of these tests, which are set forth in Example V through IX, a plating bath having the composition of Bath A of Table IV was used. As before, plating operations in each of these examples were carried out in a standard Hull test cell so that the effect of a wide range of current densities could be observed. The electrodeposits were formed on brass test panels at a temperature of 68° C. and without agitation.

#### EXAMPLE V

To the standard copper plating bath was added 0.003 gram per liter of potassium selenocyanate and 0.003 gram per liter of bismuth trioxide (as the tartarate complex). A test panel which received a copper electroplate from this bath was bright over a current density range from 1 to 8 amperes per square foot, but exhibited slight haziness in the middle current density range. Upon the addition of 30 grams per liter of potassium nitrate to this bath, the resultant electroplate was exceptionally bright

10

15

20

25

30

35

40

45

50

55

60

65

70

in the current density range from 12 to 50 amperes per square foot, and substantially as bright as before the nitrate addition in the range from about 1 to 12 amperes per square foot.

Identical results were obtained when 0.005 gram per liter of bismuth trioxide (as the sorbitol complex) was used in the plating solution in combination with the potassium selenocyanate and potassium nitrate.

#### EXAMPLE VI

Brilliant copper deposits are formed when the primary and secondary brightening agents are used in conjunction with an inorganic nitrite. The test panel of a Hull cell received a copper electrodeposit from the standard copper plating bath which contained 0.003 gram per liter of potassium selenocyanate and 0.003 gram per liter of bismuth trioxide (as the tartarate complex). The plated panel was bright at the low current density end (1 to 12 amperes per square foot). Upon adding 30 grams per liter of potassium nitrite to this bath, the copper deposit formed was exceptionally bright over the current density range corresponding to 12 to 50 amperes per square foot, and about as bright as before the nitrate addition below 12 amperes per square foot.

#### EXAMPLE VII

To a standard copper plating bath were added 0.064 gram per liter of sodium selenite and 8.8 millimoles per liter of [(N-hydroxyethyl-diethanolatoamine-O,O',N) titanium (IV)], and copper was electrodeposited on a Hull test panel. The deposit was bright over a current density range from 1 to 8 amperes per square foot, representing 35 percent of the panel. Upon the addition of 30 grams per liter of potassium nitrate to this bath, a brilliant electrodeposit was obtained over the entire panel, corresponding to a current density range from 1 to 50 amperes per square foot.

In a comparative operation, the substitution of 30 grams per liter of potassium nitrite for the potassium nitrate yielded identical results.

#### EXAMPLE VIII

Using the standard copper plating solution to which 0.003 gram per liter of potassium selenocyanate and 1 gram per liter of 2-butyne-1,4-diol had been added, a bright copper deposit was formed on a test panel in a Hull cell throughout the current density range from 1 and 22 amperes per square foot, covering about three-fifths of the panel. When, however, 30 grams per liter of potassium nitrate were added to this bath, the electrodeposit was brilliant over the full width of the panel, corresponding to a current density range from 1 to 50 amperes per square foot. Both potassium nitrite and sodium nitrite gave identical results when substituted for the potassium nitrate.

#### EXAMPLE IX

A cumulative brightening effect is also exerted on the plating bath when an oxime or nitroalkane is used in place of an inorganic nitrate or nitrite. These organic nitroxy compounds are somewhat susceptible to hydrolysis but the effect of base hydrolysis may be substantially avoided by operating the cell at lower temperatures (say near room temperature).

Using the standard copper plating bath which contained 0.003 gram per liter of potassium selenocyanate and 1 gram per liter of 2-butyne-1,4-diol, a bright copper electrodeposit was formed on the test panel of a Hull cell over the current density range of 1 to 22 amperes per square foot. Upon adding 45 grams per liter of nitromethane to this bath, the bright range has extended to about 40 amperes per square foot. Substituting an equivalent amount of acetaldoxime or dimethylglyoxime for the nitromethane similarly resulted in a substantial increase in the brightness range.

We claim:

1. A process for producing a bright copper electroplate which comprises electrodepositing copper from an aqueous alkaline cyanide copper plating bath in which there is dissolved from 0.01 to 20 millimoles per liter of an alkali-soluble selenium compound and from 0.005 to 200 millimoles per liter of a water-soluble acetylenic compound.

2. A process for producing a bright copper electroplate which comprises electrodepositing copper from an aqueous alkaline cyanide copper plating bath in which there is dissolved from 0.001 to 1 gram per liter of selenium added in the form of an alkali-soluble selenium compound, and from about 0.01 to about 100 millimoles per liter of a water-soluble acetylenic compound.

3. A process for producing a bright copper electroplate which comprises electrodepositing copper from an aqueous alkaline cyanide copper plating bath in which there is dissolved from 0.001 to 1 gram per liter of selenium added in the form of an alkali-soluble selenium compound, from about 0.01 to about 100 millimoles per liter of a water-soluble acetylenic compound, and from 5 to 60 grams per liter of an alkali-soluble nitroxy compound which, upon dissolving in alkaline solution, contains an ionic moiety represented by the formula



in which  $\alpha$  is an atom selected from the group consisting of oxygen and disubstituted carbon atoms, and  $\beta$  is a member of the group consisting of an electron pair and a coordinately bonded oxygen atom.

4. A process for producing a bright copper electroplate which comprises electrodepositing copper from an aqueous alkaline cyanide copper plating bath in which there is dissolved from 0.001 to 1 gram per liter of selenium added in the form of an alkali-soluble selenium compound, from about 0.01 to about 100 millimoles per liter of a water-soluble acetylenic compound, and from 5 to 60 grams per liter of an alkali-soluble nitroxy compound selected from the group consisting of nitroalkanes, oximes, and nitrates and nitrites of alkali metals, magnesium, ammonium and copper.

5. The process for producing a bright copper electroplate which comprises electrodepositing copper from an aqueous alkaline cyanide copper plating bath in which there is dissolved from 0.01 to 20 millimoles per liter of an alkali-soluble selenium compound and from 1 to 200 millimoles per liter of a water-soluble acetylenic compound.

6. The process for producing a bright copper electroplate which comprises electrodepositing copper from an aqueous alkaline cyanide copper plating bath in which there is dissolved from 0.01 to 20 millimoles per liter of an alkali-soluble selenium compound selected from the group consisting of selenides, selenites, selenates, and selenocyanates, and from 1 to 200 millimoles per liter of a water-soluble acetylenic compound.

7. The process for producing a bright copper electroplate which comprises electrodepositing copper from an aqueous alkaline cyanide copper plating bath in which there is dissolved from 0.01 to 20 millimoles per liter of an alkali-soluble selenium compound and from 1 to 200 millimoles per liter of a water-soluble acetylenic compound having the structure



in which  $\text{R}_1^\bullet$  and  $\text{R}_2^\bullet$  are substituents selected from the group consisting of hydrogen and alkyl and hydroxy-substituted alkyl radicals,  $\text{R}_1^\bullet$  is a substituent selected from the group consisting of hydroxy, hydroxymethyl, methoxy, hydroxyethyl, ethoxy, and hydroxyethoxy radicals, and  $\text{R}_2^\bullet$  is a substituent selected from the group consisting of hydrogen, halogen, diethylaminoethyl, morpholinomethyl, alkyl, alkenyl, alkynyl, and hydroxy-, methoxy-, and ethoxy-substituted alkyl, alkenyl, and alkynyl radicals.

8. The process for producing a bright copper electroplate which comprises electrodepositing copper from an aqueous alkaline cyanide copper plating bath in which there is dissolved from 0.01 to 20 millimoles per liter of an alkali-soluble selenium compound selected from the group consisting of selenides, selenites, selenates, and selenocyanates, from about 1 to about 200 millimoles per liter of a water-soluble acetylenic compound, and from about 5 to about 60 grams per liter of a nitroxy compound selected from the group consisting of nitroalkanes, oximes, and nitrates and nitrites of alkali metals, magnesium, ammonium, and copper.

9. The process for producing a bright copper electroplate which comprises electrodepositing copper from an aqueous alkaline cyanide copper plating bath in which there is dissolved from 0.01 to 20 millimoles per liter of an alkali-soluble selenium compound selected from the group consisting of selenides, selenites, selenates, and selenocyanates, and from about 0.1 to about 10 grams per liter of 2-butyne-1,4-diol.

10. The process for producing a bright copper electroplate which comprises electrodepositing copper from an aqueous alkaline cyanide copper plating bath in which there is dissolved from 0.01 to 20 millimoles per liter of an alkali-soluble selenium compound, from 1 to 200 millimoles per liter of a water-soluble acetylenic compound, and from about 0.05 to about 0.5 gram per liter of an alkali-soluble nitrile.

11. The process for producing a bright copper electroplate which comprises electrodepositing copper from an aqueous alkaline cyanide copper plating bath in which there is dissolved from 0.01 to 20 millimoles per liter of an alkali-soluble selenium compound, from 1 to 200 millimoles per liter of a water-soluble acetylenic compound, and from about 0.05 to about 0.5 gram per liter of a nitrile selected from the group consisting of succinonitrile, dicyandiamide,  $\beta,\beta'$ -oxydipropionitrile,  $\beta$ -sulfo-propionitrile, potassium dicyanoguanidine, and sodium dicyanamide.

#### References Cited in the file of this patent

#### UNITED STATES PATENTS

|           |          |       |               |
|-----------|----------|-------|---------------|
| 2,694,677 | Ostrow   | ----- | Nov. 16, 1954 |
| 2,770,587 | Ostrow   | ----- | Nov. 13, 1956 |
| 2,825,684 | Wernlund | ----- | Mar. 4, 1958  |

#### FOREIGN PATENTS

|         |         |       |               |
|---------|---------|-------|---------------|
| 874,100 | Germany | ----- | Apr. 20, 1953 |
| 925,490 | Germany | ----- | Mar. 3, 1955  |

#### OTHER REFERENCES

Serial No. 331,456, Weiner (A.P.C.), published July 13, 1943.

UNITED STATES PATENT OFFICE  
Certificate of Correction

Patent No. 2,881,121

April 7, 1959

Donald G. Foulke et al.

It is hereby certified that error appears in the printed specification of the above numbered patent requiring correction and that the said Letters Patent should read as corrected below.

Columns 3 and 4, line 28, Table I, second column thereof, tenth item, for

$\text{CH}_3-\text{C}(\text{CH}_3)(\text{OH})\text{C}_2\text{CH}$  read  $\text{CH}_3-\text{C}(\text{CH}_3)(\text{OH})\text{C}\equiv\text{CH}$

column 3, line 70, for "organic" read —inorganic—; column 5, lines 47 to 52, Table II, second column thereof should appear as shown below instead of as in the patent:

0.05 to 0.5  
0.12 to 0.5  
0.12 to 0.5  
0.12 to 0.5  
0.12 to 0.5  
0.12 to 0.5

column 8, line 71, for "has" read —was—; column 9, lines 26 to 28, the formula should appear as shown below instead of as in the patent:



column 10, line 60, list of references cited, under "FOREIGN PATENTS", for "925,490 Germany ----- Mar. 3, 1955" read —924,490 Germany ----- Mar. 3, 1955—.

Signed and sealed this 28th day of July 1959.

[SMAL]

Attest:

KARL H. AXLINE,  
*Attesting Officer.*

ROBERT C. WATSON,  
*Commissioner of Patents.*